

1

3,677,744

### AGE HARDENING STAINLESS STEEL

Katsumi Yamamura, Hiroshi Harigaya, and Kazutomo Kasai, Suwa-shi, and Michio Asahina, Okaya-shi, Japan, assignors to Kabushiki Kaisha Suwa Seikosha, Tokyo, Japan

No Drawing. Filed Dec. 9, 1968, Ser. No. 782,431  
Claims priority, application Japan, Mar. 7, 1968,

43/14,498; Mar. 19, 1968, 43/17,689

Int. Cl. C22c 13/20

U.S. Cl. 75—128 T

6 Claims 10

#### ABSTRACT OF THE DISCLOSURE

Corrosion and heat resistance, workability and toughness of age-hardenable Fe-Mo alloys are improved by the addition of Cr, Ni and Co. The age hardenability is reinforced by the addition of W, Be, Ti and Si. Resistance to non-oxidizing acids is improved by addition of Cu.

#### DETAILED DESCRIPTION OF INVENTION

The present invention relates to an alloy with a body centered cubic structure having high strength and high resistance to corrosion in which resistance to corrosion, workability, toughness and resistance to heat are increased by adding Cr, Ni and Co to Fe-Mo ageing alloy and ageing property is reinforced by adding W, Be and Ti. The object of the invention is to provide a relatively inexpensive alloy with high strength as construction material and spring material which require high resistance to corrosion.

It is well known that age hardening appears by adding Mo to Fe by more than 15%. Such alloys, however, can be used only as cast alloy because it is impossible to apply such work as rolling and drawing, besides its resistance to corrosion is insufficient.

On the other hand, our invention is characterized by the fact that resistance to corrosion is greatly increased by adding Cr to Fe-Mo alloy, and the amount of Mo required for age hardening is reduced and sufficient workability can be obtained.

Further it is found that toughness, resistance to heat, resistance to corrosion are increased without spoiling the age hardening of the material by adding Co and Ni, singly or complexed, to Fe-Mo-Cr alloy, and that age hardening property is greatly increased by adding W, Be and Ti.

Composition of this alloy will be disclosed in the following.

##### (1) Cr—6 to 22%

Cr stabilizes Fe material, and increases resistance to corrosion of the material. In the alloy according to the invention, too, Cr is added to increase resistance to corrosion, the amount of Mo of Fe-Mo age hardening alloy is decreased by adding Cr. Thus workability for cold rolling and drawing etc. is improved without spoiling age hardenability. With Cr less than 6% in content resistance to corrosion is insufficient, with Cr over 22% in content the material tends to harden and spoils the workability.

##### (2) Mo+W—4 to 13% ( $\frac{W}{Mo+W} \leq 0.6$ )

Element Mo in Fe-Mo alloy produces age hardening effect. The alloy according to our invention improves not only age hardening but also resistance to corrosion against non-oxidized acid. Element W in Fe material, like as Mo,

2

shows age hardening property. The effect of W on age hardening property is weaker than that of Mo. However, it shows greater reinforcement for solid solution than Mo, so it strengthens the matrix of this alloy. Too much addition, however, makes the material brittle and deteriorates its workability. After examined each alloy from three points, i.e. age hardenability, solid solution reinforcement, brittleness of the material, it was found that Mo+W should be 4 to 13%, W being up to 60% of the total amount added.

##### (3) Co-Ni

|                     | Percent                 |
|---------------------|-------------------------|
| Co only             | 0.5 to 12.              |
| Ni only             | From 0.5 up to 5.       |
| Co and Ni complexed | 0.5 to 12. <sup>1</sup> |

<sup>1</sup> Ni less than 4.5%.

Co and Ni greatly increase toughness of the material and improve workability of rolling and drawing. These elements improve resistance to corrosion. Especially Ni improves resistance to corrosion at normal temperature and Co improves acid proofness at high temperature. The amounts added should be as described above. When the amounts added is less than the lower limit, there is little effect and when the amount exceeds the upper limit, the material tends to brittle and workability deteriorates. Ni with more than 5% added, tends to produce  $\gamma$  phase, therefore too much addition should be avoided.

##### (4) Ti-Be

|                     | Percent     |
|---------------------|-------------|
| Ti only             | 0.1 to 4    |
| Be only             | 0.05 to 2   |
| Ti and Be complexed | 0.05 to 3.5 |

Ti and Be in Fe material stabilize ferrite. With the lowering of the temperature, its solubility decreases and age hardening effect appears. The alloy according to the invention has body centered, ferrite crystal construction. By means of these elements strength is greatly increased without spoiling its hardenable property. This great effect is due to the fact that treatment condition for hard ageing of Fe-Mo and that of Fe-Be and Fe-Ti are similar, and that the precipitation compounds which contribute to hardening have completely different phases and not influence with each other. Therefore Ti and Be added together do not spoil the hardening effect. When the amount added is less than the lower limit, hardenability deteriorates and when the amount added of Ti and Be, singly or mixed together is over the upper limit, the material becomes brittle and working becomes difficult.

##### (5) Si—less than 2%

Si deoxidizes melting metal and promotes ageing of Fe-Mo alloy. With Si more than 0.5% in content age hardening appears. However when the amount of Si exceeds 2%, the material tends to be brittle.

##### (6) Cu—less than 3%

Cu improves proofness against non-oxidized acid. It also shows age hardening effect. Too much addition, however, deteriorates workability, especially hot workability, and resistance to corrosion. After various experiments it was found that Cu less than 3% in content is most suitable.

##### (7) Nb—less than 0.3%

Nb reacts with C to form stable carbide and improves resistance to corrosion. Particularly in this alloy, Ti, Mo and Cr easily reacts with C and deteriorates not only

resistance to corrosion but also age hardenability. By adding Nb, carbide of Nb stable at higher temperature is formed, which prevents the reaction with these elements. However, when Nb is added by more than 0.3%, it tends to form compound with other elements than C, and brittleness of the material increases.

(8) C—less than 0.1%

C easily forms carbide with Mo, Ti and Cr, and deteriorates resistance to corrosion and age hardenability. C should be avoided as much as possible, but it is inevitably intermingled during melting operation. Considering the above fact, Nb is added in the present alloy. Nb of less than 0.1% in content is sufficient.

Referring now to the embodiment of the invention, Table 1 shows a typical composition of the alloy according to the present invention. For comparison, two kinds of age hardening stainless steel on the market and that of 18-8 stainless steel are also shown.

In Table 1, all alloys Nos. 1 to 33 were melted in vacuum by high frequency induction furnace wherein degree of vacuum in melting was maintained at 3 to  $8 \times 10^{-3}$  mm. Hg. Such melting material as electrolytic pure iron, pure Cr, Ferro-Mo, Ferro-W, pure Co, pure Ni, Ferro-Ti, Ferro-Be, Ferro-Nb, Ferro-Si, electrolytic pure copper were used. They were melted in such a manner that electrolytic pure iron, pure Cr, Ferro-Mo, Ferro-W, pure Co, pure Ni were charged in high pure alumina crucible and the furnace was made vacuous, then the melting operation was started. Added Fe-Si after the material was melted down in the crucible. The temperature was set to the value 100 to 200° C. above the melting temperature when the melting metal became clean. Threw in quickly Cu, Ferro-Nb, Ferro-Ti and Ferro-Be in this order. One or two minutes after Ferro-Be was melted, ingot was cast. The temperature was measured by optical pyrometer. Surface of these ingots were made smooth and band material was formed by hot forging, hot and cold rolling, i.e. hot rolling at 1050 to 900° C. and heated up to 1150 to 1200° C. and quenched by water to be used for test pieces for strength and resistance to corrosion.

4

Table 2 shows hardness, tensile strength and elongation of these alloys. From this result, it can be seen that addition of Ni or Co has great influence on toughness of the material. Alloys from Nos. 17 to 33 have higher elongation than those from Nos. 1 to 16 which do not include Ni and Co. Alloys including such age hardening elements as Ti or Be, show higher hardness in melting than those which do not include them. These alloys when melting have the same strength as 17-4 PH and 17-7 PH on the market which are known as age hardening stainless steel.

TABLE 2.—STRENGTH OF MELTING MATERIAL

|                        | Hardness<br>(Hv) | Tensile strength<br>(kg./mm. <sup>2</sup> ) | Elongation<br>(percent) |
|------------------------|------------------|---------------------------------------------|-------------------------|
| 1                      | 262              | 102                                         | 8                       |
| 2                      | 250              | 96                                          | 11                      |
| 3                      | 266              | 93                                          | 10                      |
| 4                      | 242              | 91                                          | 15                      |
| 5                      | 248              | 95                                          | 14                      |
| 6                      | 246              | 98                                          | 13                      |
| 7                      | 271              | 100                                         | 12                      |
| 8                      | 255              | 94                                          | 11                      |
| 9                      | 302              | 103                                         | 10                      |
| 10                     | 318              | 102                                         | 9                       |
| 11                     | 310              | 101                                         | 12                      |
| 12                     | 298              | 98                                          | 12                      |
| 13                     | 268              | 102                                         | 10                      |
| 14                     | 311              | 103                                         | 11                      |
| 15                     | 306              | 99                                          | 12                      |
| 16                     | 314              | 103                                         | 8                       |
| 17                     | 322              | 101                                         | 27                      |
| 18                     | 318              | 108                                         | 24                      |
| 19                     | 286              | 96                                          | 18                      |
| 20                     | 291              | 103                                         | 34                      |
| 21                     | 334              | 111                                         | 26                      |
| 22                     | 280              | 102                                         | 31                      |
| 23                     | 301              | 98                                          | 20                      |
| 24                     | 306              | 104                                         | 27                      |
| 25                     | 287              | 103                                         | 30                      |
| 26                     | 298              | 106                                         | 31                      |
| 27                     | 300              | 101                                         | 29                      |
| 28                     | 311              | 108                                         | 26                      |
| 29                     | 294              | 105                                         | 29                      |
| 30                     | 281              | 99                                          | 30                      |
| 31                     | 301              | 103                                         | 26                      |
| 32                     | 311              | 116                                         | 24                      |
| 33                     | 298              | 108                                         | 28                      |
| Alloys to be compared: |                  |                                             |                         |
| 17-4 PH                | 370              | 105                                         | 12                      |
| 17-7 PH                | 183              | 91                                          | 35                      |
| 18-8                   | 153              | 60                                          | 50                      |

TABLE 1

|                                    | Cr | Mo | W | Co    | Ni    | Ti   | Be    | Si   | Cu   | Nb   | C    | Fe       |      |
|------------------------------------|----|----|---|-------|-------|------|-------|------|------|------|------|----------|------|
| Alloys according to the invention: |    |    |   |       |       |      |       |      |      |      |      |          |      |
| 1                                  |    |    |   | 8.03  | 11.12 |      |       | 0.48 |      | 0.10 | 0.02 | Balance. |      |
| 2                                  |    |    |   | 10.12 | 9.98  |      |       | 0.29 | 2.50 |      | 0.02 | Do.      |      |
| 3                                  |    |    |   | 12.06 | 9.11  |      |       | 0.31 | 2.49 | 0.21 | 0.03 | Do.      |      |
| 4                                  |    |    |   | 14.96 | 5.89  |      |       | 2.33 | 2.91 |      | 0.02 | Do.      |      |
| 5                                  |    |    |   | 15.00 | 8.01  |      |       | 0.03 | 1.01 | 0.12 | 0.02 | Do.      |      |
| 6                                  |    |    |   | 15.10 | 9.08  |      |       | 1.02 | 1.04 | 0.11 | 0.02 | Do.      |      |
| 7                                  |    |    |   | 20.05 | 10.05 |      |       |      |      |      | 0.03 | Do.      |      |
| 8                                  |    |    |   | 20.12 | 7.20  |      |       |      |      |      | 0.02 | Do.      |      |
| 9                                  |    |    |   | 6.33  | 7.21  | 3.58 |       | 0.28 | 2.55 |      | 0.02 | Do.      |      |
| 10                                 |    |    |   | 7.82  | 11.31 |      |       | 1.35 |      | 0.10 | 0.02 | Do.      |      |
| 11                                 |    |    |   | 8.45  | 5.08  | 4.12 |       | 0.23 | 0.36 | 0.42 | 2.01 |          |      |
| 12                                 |    |    |   | 11.27 | 8.47  |      |       | 1.04 | 0.22 |      | 0.13 | 0.02     |      |
| 13                                 |    |    |   | 12.58 | 5.27  | 4.18 |       |      | 1.67 | 2.85 | 0.08 | 0.03     |      |
| 14                                 |    |    |   | 14.75 | 8.46  |      |       | 0.16 | 0.82 | 0.76 |      | 0.10     |      |
| 15                                 |    |    |   | 16.12 | 6.22  |      |       |      | 1.62 | 0.34 | 1.15 | 0.09     |      |
| 16                                 |    |    |   | 18.38 | 9.65  | 0.28 |       | 0.72 | 0.21 | 0.48 |      | 0.02     |      |
| 17                                 |    |    |   | 6.36  | 7.14  | 3.50 |       | 2.28 | 1.42 |      | 1.08 | 0.02     |      |
| 18                                 |    |    |   | 8.36  | 10.92 |      |       | 4.59 |      | 1.41 | 0.42 | 0.11     |      |
| 19                                 |    |    |   | 11.91 | 8.10  | 1.23 |       | 0.83 | 0.23 | 0.38 | 0.22 | 1.00     |      |
| 20                                 |    |    |   | 15.11 | 9.01  |      |       | 4.23 | 0.13 | 0.03 | 0.91 | 0.85     |      |
| 21                                 |    |    |   | 19.42 | 8.63  | 1.37 |       | 3.25 | 2.04 | 0.13 | 0.38 | 0.62     |      |
| 22                                 |    |    |   | 15.03 | 9.03  |      |       | 4.72 |      | 1.08 | 0.96 | 0.12     |      |
| 23                                 |    |    |   | 8.55  | 9.57  | 1.14 | 0.92  | 1.23 | 0.33 | 0.42 | 1.16 |          |      |
| 24                                 |    |    |   | 10.34 | 5.64  | 4.62 | 3.66  |      | 1002 | 0.64 |      | 0.13     |      |
| 25                                 |    |    |   | 15.01 | 8.89  |      | 5.12  |      |      | 1.02 | 1.00 | 0.11     |      |
| 26                                 |    |    |   | 18.42 | 6.03  | 3.28 | 7.08  |      | 0.42 |      | 0.96 | 0.85     |      |
| 27                                 |    |    |   | 7.21  | 11.01 |      | 9.32  |      | 1.88 | 0.09 | 0.23 |          |      |
| 28                                 |    |    |   | 14.96 | 7.28  | 1.03 | 11.02 |      | 2.18 |      | 0.34 | 0.66     |      |
| 29                                 |    |    |   | 7.15  | 10.86 |      | 6.14  | 2.03 | 0.89 |      | 1.23 | 1.07     |      |
| 30                                 |    |    |   | 10.77 | 8.11  | 1.30 | 2.26  | 3.18 |      | 0.30 | 0.41 | 0.12     |      |
| 31                                 |    |    |   | 15.18 | 9.02  | 0.84 | 9.22  | 1.05 |      |      | 0.96 | 0.88     |      |
| 32                                 |    |    |   | 17.45 | 6.03  | 4.35 | 1.12  | 4.36 | 1.89 | 0.16 | 0.14 | 0.35     |      |
| 33                                 |    |    |   | 19.05 | 4.58  | 4.72 | 4.26  | 2.16 | 0.43 |      | 1.19 | 0.92     |      |
| Alloys compared:                   |    |    |   |       |       |      |       |      |      |      |      |          |      |
| 17-4 PH                            |    |    |   | 16.88 |       |      |       | 4.13 | 0.21 | 0.62 | 4.01 | 6.81     | 0.05 |
|                                    |    |    |   |       |       |      |       |      |      | Al   |      |          |      |
| 17-7 PH                            |    |    |   | 17.00 |       |      |       | 7.11 |      | 1.15 | 0.83 |          | 0.67 |
| 18-8                               |    |    |   | 18.54 |       |      |       | 8.91 |      |      | 0.48 |          | 0.96 |

Table 3 shows hardness and tensile strength of 50% cold rolled material and those when this alloy is aged. Age hardening treatment was performed both in the alloy according to the invention and the material compared under such a condition that the maximum strength was obtained in the preliminary experiment. All heat treatment was performed in the vacuum furnace in order to avoid oxidation. From the results shown in Table 3, it can be seen that before age hardening treatment there is little difference between the alloys according to the invention and the alloys compared, 17-4 PH, 17-7 PH and 18-8 stainless steel, but that there appears great difference between them after aged, which shows that the ageing property of the alloys according to the invention is excellent.

After age hardening treatment test pieces in Table 3 were immersed in various corrosion liquids for ten days and its degree of corrosion and discoloration was examined. The results are shown in Table 4.

TABLE 3

| Alloys according to the invention | 50% rolled material                      |               |                  | Age hardening material                   |               |    |
|-----------------------------------|------------------------------------------|---------------|------------------|------------------------------------------|---------------|----|
|                                   | Tensile strength (kg./mm. <sup>2</sup> ) | Hardness (HV) | Ageing condition | Tensile strength (kg./mm. <sup>2</sup> ) | Hardness (HV) |    |
| 1                                 | 122                                      | 342           | 570° C. X7H      | 205                                      | 720           |    |
| 2                                 | 128                                      | 391           | Same as above    | 195                                      | 662           |    |
| 3                                 | 129                                      | 389           | do               | 192                                      | 641           |    |
| 4                                 | 126                                      | 360           | do               | 191                                      | 638           |    |
| 5                                 | 116                                      | 341           | do               | 196                                      | 582           |    |
| 6                                 | 125                                      | 347           | do               | 198                                      | 656           |    |
| 7                                 | 132                                      | 418           | do               | 183                                      | 497           |    |
| 8                                 | 120                                      | 392           | do               | 178                                      | 420           |    |
| 9                                 | 152                                      | 428           | do               | 237                                      | 762           |    |
| 10                                | 148                                      | 412           | do               | 218                                      | 723           |    |
| 11                                | 150                                      | 419           | do               | 241                                      | 723           |    |
| 12                                | 146                                      | 408           | do               | 219                                      | 736           |    |
| 13                                | 134                                      | 395           | do               | 216                                      | 636           |    |
| 14                                | 144                                      | 415           | do               | 224                                      | 741           |    |
| 15                                | 142                                      | 421           | do               | 223                                      | 743           |    |
| 16                                | 144                                      | 406           | do               | 219                                      | 732           |    |
| 17                                | 150                                      | 431           | do               | 228                                      | 758           |    |
| 18                                | 152                                      | 428           | do               | 222                                      | 749           |    |
| 19                                | 150                                      | 419           | do               | 240                                      | 756           |    |
| 20                                | 137                                      | 368           | do               | 209                                      | 707           |    |
| 21                                | 158                                      | 449           | do               | 238                                      | 752           |    |
| 22                                | 134                                      | 352           | do               | 201                                      | 694           | 40 |
| 23                                | 148                                      | 412           | do               | 202                                      | 740           |    |

TABLE 3—Continued

| 5       | Alloys according to the invention | 50% rolled material                      |               |                  | Age hardening material                   |               |
|---------|-----------------------------------|------------------------------------------|---------------|------------------|------------------------------------------|---------------|
|         |                                   | Tensile strength (kg./mm. <sup>2</sup> ) | Hardness (HV) | Ageing condition | Tensile strength (kg./mm. <sup>2</sup> ) | Hardness (HV) |
| 24      |                                   | 150                                      | 420           | 570° C. X7H      | 216                                      | 681           |
| 25      |                                   | 139                                      | 371           | Same as above    | 203                                      | 694           |
| 26      |                                   | 146                                      | 395           | do               | 223                                      | 706           |
| 27      |                                   | 153                                      | 419           | do               | 221                                      | 736           |
| 28      |                                   | 180                                      | 431           | do               | 229                                      | 743           |
| 29      |                                   | 132                                      | 385           | do               | 214                                      | 605           |
| 30      |                                   | 129                                      | 361           | do               | 199                                      | 705           |
| 31      |                                   | 138                                      | 392           | do               | 208                                      | 682           |
| 32      |                                   | 143                                      | 396           | do               | 224                                      | 703           |
| 33      |                                   | 136                                      | 389           | do               | 217                                      | 701           |
| 17-4 PH |                                   | 120                                      | 380           | H900             | 150                                      | 430           |
| 17-7 PH |                                   | 140                                      | 420           | CH900            | 183                                      | 500           |
| 18-8    |                                   | 140                                      | 385           |                  |                                          |               |

Artificial sea water and artificial sweat in Table 4 are sweat and sea water made artificially by mixing chemicals, the components of which are similar to those of natural sweat and sea water. Their compositions are as follows:

| 25 | Component of artificial sweat:     | Percent          |
|----|------------------------------------|------------------|
|    | NaCl                               | 0.648 to 0.987   |
| 30 | Na <sub>2</sub> S                  | 0.006 to 0.025   |
|    | (NH <sub>2</sub> ) <sub>2</sub> Co | 0.086 to 0.173   |
|    | NH <sub>4</sub> OH                 | 0.010 to 0.018   |
|    | Saccharose                         | 0.006 to 0.022   |
|    | Lactic acid                        | 0.034 to 0.107   |
| 35 | Component of artificial sea water: |                  |
|    | NaCl                               | 2.30 to 2.35     |
|    | MgCl <sub>2</sub>                  | 0.45 to 0.49     |
|    | Na <sub>2</sub> SO <sub>4</sub>    | 0.37 to 0.39     |
|    | CaCl <sub>2</sub>                  | 0.10 to 0.12     |
|    | KCl                                | 0.063 to 0.066   |
|    | NaHCO <sub>3</sub>                 | 0.018 to 0.020   |
|    | KBr                                | 0.0080 to 0.0095 |

TABLE 4

|                          | Artificial sweat | Artificial sea water | 10% NaCl | 10% HCl | 5% H <sub>2</sub> SO <sub>4</sub> | 10% NH <sub>4</sub> Cl | 10% NH <sub>4</sub> OH | 5% Na <sub>2</sub> S | 10% lactic acid | 20% Na <sub>2</sub> CO <sub>3</sub> |
|--------------------------|------------------|----------------------|----------|---------|-----------------------------------|------------------------|------------------------|----------------------|-----------------|-------------------------------------|
| 1                        | ○                | ○                    | △        | ○       | △                                 | ○                      | ○                      | ○                    | ○               | ○                                   |
| 2                        | ○                | ○                    | △        | ○       | △                                 | ○                      | ○                      | ○                    | ○               | ○                                   |
| 3                        | ○                | ○                    | △        | ○       | △                                 | ○                      | ○                      | ○                    | ○               | ○                                   |
| 4                        | ○                | ○                    | △        | ○       | △                                 | ○                      | ○                      | ○                    | ○               | ○                                   |
| 5                        | ○                | ○                    | ○        | ○       | ○                                 | ○                      | ○                      | ○                    | ○               | ○                                   |
| 6                        | ○                | ○                    | ○        | ○       | ○                                 | ○                      | ○                      | ○                    | ○               | ○                                   |
| 7                        | ○                | ○                    | ○        | ○       | ○                                 | ○                      | ○                      | ○                    | ○               | ○                                   |
| 8                        | ○                | ○                    | ○        | ○       | ○                                 | ○                      | ○                      | ○                    | ○               | ○                                   |
| 9                        | ○                | ○                    | ○        | ○       | ○                                 | ○                      | ○                      | ○                    | ○               | ○                                   |
| 10                       | ○                | ○                    | △        | ○       | △                                 | ○                      | ○                      | ○                    | ○               | ○                                   |
| 11                       | ○                | ○                    | △        | ○       | △                                 | ○                      | ○                      | ○                    | ○               | ○                                   |
| 12                       | ○                | ○                    | △        | ○       | △                                 | ○                      | ○                      | ○                    | ○               | ○                                   |
| 13                       | ○                | ○                    | △        | ○       | △                                 | ○                      | ○                      | ○                    | ○               | ○                                   |
| 14                       | ○                | ○                    | ○        | ○       | ○                                 | ○                      | ○                      | ○                    | ○               | ○                                   |
| 15                       | ○                | ○                    | ○        | ○       | ○                                 | ○                      | ○                      | ○                    | ○               | ○                                   |
| 16                       | ○                | ○                    | ○        | ○       | ○                                 | ○                      | ○                      | ○                    | ○               | ○                                   |
| 17                       | ○                | ○                    | ○        | ○       | ○                                 | ○                      | ○                      | ○                    | ○               | ○                                   |
| 18                       | ○                | ○                    | ○        | ○       | ○                                 | ○                      | ○                      | ○                    | ○               | ○                                   |
| 19                       | ○                | ○                    | ○        | ○       | ○                                 | ○                      | ○                      | ○                    | ○               | ○                                   |
| 20                       | ○                | ○                    | ○        | ○       | ○                                 | ○                      | ○                      | ○                    | ○               | ○                                   |
| 21                       | ○                | ○                    | ○        | ○       | ○                                 | ○                      | ○                      | ○                    | ○               | ○                                   |
| 22                       | ○                | ○                    | ○        | ○       | ○                                 | ○                      | ○                      | ○                    | ○               | ○                                   |
| 23                       | ○                | ○                    | ○        | ○       | ○                                 | ○                      | ○                      | ○                    | ○               | ○                                   |
| 24                       | ○                | ○                    | ○        | ○       | ○                                 | ○                      | ○                      | ○                    | ○               | ○                                   |
| 25                       | ○                | ○                    | ○        | ○       | ○                                 | ○                      | ○                      | ○                    | ○               | ○                                   |
| 26                       | ○                | ○                    | ○        | ○       | ○                                 | ○                      | ○                      | ○                    | ○               | ○                                   |
| 27                       | ○                | ○                    | ○        | ○       | ○                                 | ○                      | ○                      | ○                    | ○               | ○                                   |
| 28                       | ○                | ○                    | ○        | ○       | ○                                 | ○                      | ○                      | ○                    | ○               | ○                                   |
| 29                       | ○                | ○                    | ○        | ○       | ○                                 | ○                      | ○                      | ○                    | ○               | ○                                   |
| 30                       | ○                | ○                    | ○        | ○       | ○                                 | ○                      | ○                      | ○                    | ○               | ○                                   |
| 31                       | ○                | ○                    | ○        | ○       | ○                                 | ○                      | ○                      | ○                    | ○               | ○                                   |
| 32                       | ○                | ○                    | ○        | ○       | ○                                 | ○                      | ○                      | ○                    | ○               | ○                                   |
| 33                       | ○                | ○                    | ○        | ○       | ○                                 | ○                      | ○                      | ○                    | ○               | ○                                   |
| 17-4 PH                  | △                | △                    | △        | △       | X                                 | X                      | X                      | ○                    | ○               | ○                                   |
| 17-7 PH                  | △                | △                    | △        | △       | X                                 | X                      | X                      | ○                    | ○               | ○                                   |
| 18-8 50% rolled material | ○                | ○                    | △        | △       | △                                 | △                      | ○                      | ○                    | ○               | ○                                   |

NOTE.—○=No discoloration or corrosion; △=Discoloration and slight corrosion; ○=Slight discoloration; X=Corrosion.

From Table 4 it can be seen that the alloys according to the invention have higher corrosion resistance than 17-4 PH and 17-7 PH which are known as age hardening stainless steel. It shows similar resistance to corrosion with that of 18-8 stainless steel which has high work hardenability.

As described above, the alloy according to the invention has excellent age hardenability and corrosion resistance and is suitable as the construction members for machine and spring members, in which high corrosion resistance is required.

What we claim is:

1. Age-hardenable, corrosion-resistant stainless steel, consisting essentially of 6-20% Cr, 4-12% of Mo+W, the ratio of W to Mo+W being up to 0.6, 0.5-5% Ni, up to 2% of Si, up to 3% of Cu, carbon is present in an amount up to 0.1% Nb in quantity sufficient only to form carbide with substantially all of the carbon present, but in any case less than 0.3% and a metal selected from the group consisting of Ti, Be and mixtures thereof, where the Ti content in the absence of Be is in the range of 0.1-4%, the Be content in the absence of Ti is in the range of 0.05-2%, and the total Ti+Be content when introduced as said mixture is in the range 0.05-3.5%, the balance being Fe.

2. Age-hardenable, corrosion-resistant stainless steel consisting essentially of about 6.4% Cr, about 7.1% Mo, about 3.5% W, about 2.3% Ni, about 1.4% Ti, about 0.3% Si, about 1.1% Cu, about 0.02% C, the remainder being Fe.

3. Age-hardenable, corrosion-resistant stainless steel consisting essentially of about 8.4% Cr, about 10.9% Mo, about 4.6% Ni, about 1.4% Be, about 0.4% Si, about 0.1% Nb, and about 0.02% C, the balance being Fe.

4. Age-hardenable, corrosion-resistant stainless steel

consisting essentially of about 11.9% Cr, about 8.1% Mo, about 1.2% W, about 0.8% Ni, about 0.2% Ti, about 0.4% Be, about 0.2% Si, about 1.0% Cu, about 0.1% Nb, and about 0.02% C, the balance being Fe.

5. Age-hardenable, corrosion-resistant stainless steel consisting essentially of about 19.4% Cr, about 8.6% Mo, about 1.4% W, about 3.2% Ni, about 2.0% Ti, about 0.1% Be, about 0.4% Si, about 0.6% Cu, and about 0.02% C, the balance being Fe.

10 6. Stainless steel as defined in claim 1, wherein said Mo content is 4-12%, said W content is 0-7.2%, said Si content is 0.2-2%, said Cu content is 0.5-3.0%, and said C content is 0-0.1%.

#### References Cited

#### UNITED STATES PATENTS

|           |         |          |          |
|-----------|---------|----------|----------|
| 1,587,614 | 6/1926  | Strauss  | 75-128 W |
| 2,185,996 | 1/1940  | Hatfield | 75-128 W |
| 2,747,989 | 5/1956  | Kirkby   | 75-128 W |
| 3,152,934 | 10/1964 | Lula     | 75-128 W |
| 3,154,412 | 10/1964 | Kasak    | 75-128 W |
| 3,235,417 | 2/1966  | Roy      | 75-128 W |
| 3,365,343 | 1/1968  | Vordahl  | 75-128 V |
| 1,968,966 | 8/1934  | Smith    | 75-126 G |
| 2,183,715 | 12/1939 | Franks   | 75-126 C |
| 2,403,141 | 7/1946  | Touceda  | 75-126 G |
| 2,875,042 | 2/1959  | Kegerise | 75-126 D |
| 2,881,236 | 4/1959  | Evrgets  | 75-126 C |
| 2,905,577 | 9/1959  | Harris   | 75-126 C |

HYLAND BIZOT, Primary Examiner

U.S. CL. X.R.

75-128 T, 128 W, 125